

# UNITED STATES PATENT OFFICE.

ARSENIO FERRER MENDEZ, OF CAMAJUANI, CUBA.

## LIQUID POLISH.

1,352,015.

Specification of Letters Patent. Patented Sept. 7, 1920.

No Drawing.

Application filed December 6, 1919. Serial No. 343,041.

To all whom it may concern:

Be it known that I, ARSENIO FERRER MENDEZ, a citizen of the Republic of Cuba, and resident at Camajuani, Province of Santa Clara, Cuba, whose post-office address is Agricultura and Martí streets, Camajuani, Province of Santa Clara, Cuba, have invented certain new and useful Improvements in Liquid Polish, of which the following is a specification.

This invention relates to an article of manufacture and its object is to provide as a new article of manufacture a liquid for polishing and burnishing surfaces of furniture, carriages and all kind of goods made of wood or metal and painted in dull shades.

The article is substantially composed of alcohol, gum-lac, linseed oil, banana spirit and camphor in various proportions.

20 The manufacture of the article is effected by merely mixing up in proper receptacles the linseed oil and banana spirit and adding thereafter the gum-lac and camphor previously dissolved in alcohol.

25 As an example of the most convenient proportion for mixing up these ingredients, the following is given: linseed oil 47 liters, banana spirit (banana juice fermented and distilled) 3 liters.

30 Dissolving then in fifty liters of alcohol 16 pounds of gum-lac and three liters of camphor and adding this solution to the two ingredients above mentioned.

In case the liquid is to be applied to very porous surfaces, to the above ingredients 35 can be added, in order to fill the pores thereof, a solution in alcohol of sandarac-resin together with ten pounds of gum-lac and three pounds of camphor (measured by dry measure), the sandarac-resin in the proportion of three pounds, and adding four pounds of powdered pumice-stone to the solution. Instead of the linseed oil any other 40 drying oil can be used. The product obtained in either case is a liquid of amber 45 color and is applied with a cloth wet in said liquid to the surface to be polished and burnished, rubbing it then with a dry puff of cotton or flannel or wool, or by any other 50 similar method to that end.

Having thus described my invention and the manner in which same is carried out, what I claim is:

1. As a new article of manufacture a liquid comprising a drying oil, alcohol, banana 55 spirit, camphor and gum-lac.

2. As a new article of manufacture a liquid comprising linseed oil, banana spirit, alcohol, gum-lac and camphor.

3. As a new article of manufacture a liquid composed of linseed oil, alcohol, banana spirit, gum-lac, camphor, sandarac-resin and powdered pumice-stone.

In witness whereof I affix my signature.

ARSENIO FERRER MENDEZ.